

## UNITED STATES PATENT OFFICE

2,416,890

## MANUFACTURE OF FIBERS AND FOILS

Joachim Amende and Willibald Ender, Ludwigshafen-on-the-Rhein, Germany; vested in the Attorney General of the United States

No Drawing. Application April 6, 1940, Serial No. 328,374. In Germany March 29, 1939

12 Claims. (Cl. 18—54)

**1** This invention relates to the manufacture of fibers and foils.

It is an object of this invention to produce fibers and foils of special properties.

A further object is to produce these fibers and foils from viscose solutions treated with superpolyamides.

A still further object is the provision of fibers and foils from ammoniacal copper oxyde solutions treated with superpolyamides.

These and other objects will appear from the detailed specification following hereinafter.

It has been found that fibers and foils of excellent properties are obtained, if solutions of viscose and cellulose in ammoniacal copper oxyde treated with alkali-soluble superpolyamides containing sulfamide groups, are spun or worked up into foils. Alkali-soluble superpolyamides are obtained according to the German patent application I. 64,124 IVd/120, filed March 20, 1939, by condensing diamines containing sulfamide groups and/or dicarboxylic acids or their functional derivatives or salts of these acids with the diamines or amino carboxylic acids containing sulfamide groups or their functional derivatives, especially lactams.

According to the description in said German application, the starting materials containing sulfamide groups can be employed in the quantities necessary for the condensation. However, a part of these starting materials may be substituted by corresponding starting materials free of sulfamide groups. It is necessary, however, that the final product have a certain content of sulfamide groups, to obtain a ready alkali-solubility. The quantity of the starting material containing sulfamide groups required for this process varies depending upon the chemical property of the starting material and can be easily determined by test.

The manufacture of the condensation products is carried out in the manner conventional for superpolyamides, especially by heating the starting materials to high temperatures in the presence or in the absence of solvents or diluents.

The superpolyamides obtained are practically colorless, resin-free substances which can be

**2** sulfamide groups. Due to this property they are suited especially for the refining of textile fibers, particularly as sizing agents. It is likewise possible to treat fibers or fabrics of textile materials with solutions of these superpolyamides, whereby the fibers or fabrics are refined with respect to their color. The fabrics or fibers of cellulose filaments thus treated absorb much more easily substantive dyestuffs and can be dyed even with acid dyestuffs, for example wool dyestuffs, and also with acetate rayon dyestuffs.

In the present invention, solutions of viscose or of cellulose in ammoniacal copper oxyde are preferably mixed with alkaline solutions of these superpolyamides and then spun in a known manner or worked up into foils. Hereby the usual coagulation agents like salt solutions or acids may be employed. The quantity of the superpolyamides, to be given to the spinning solution, may vary within wide limits. Preferably there are added not less than 5 per cent superpolyamide (related to cellulose), as otherwise the admixture of superpolyamides is of no practical value. On the other hand a multiple of superpolyamide compared with cellulose may be employed.

The fibers obtained are faster to wrinkling and possess a far higher "Bauschelastizität" (bolster-elasticity) and a more elastic grip than viscose-fibers. The grip, moreover, on account of the good "Bauschelastizität" resembles wool. Also the dyeing properties of the fibers and foils thus obtained are better than those of fibers and foils from pure viscose or pure ammoniacal copper oxyde cellulose. They absorb dyestuffs for instance much easier and can be dyed in darker shades than pure viscose or pure ammoniacal copper oxyde cellulose. Contrary to these they may be dyed with acid dyestuffs, for instance with wool dyestuffs and also with acetate silk dyestuffs. On account of the excellent dyeing properties the fibers are very much adapted for the manufacture of mixed fabrics.

*Example I*

50 parts by weight of N,N'-di-propanecarboxylic-acid-p-sulfo-benzoic-acid-amide



and 8 parts by weight of hexamethylenediamine are intimately mixed and heated for one hour to 180° and for 2 hours to 240°. The water formed is distilled off. The condensation product obtained after solidification exhibits a slightly yel-

55 spun into filaments in the molten state in a manner similar to that used for the known superpolyamides. The superpolyamides obtained are soluble in aqueous alkalies in contrast to the known superpolyamides which do not contain

lowish color and is soluble in a concentrated aqueous alkali solution. It can be drawn into filaments in the molten state.

A 20 per cent solution of said superpolyamide consisting of hexamethylenediamine and N.N'-dipropane-carboxylic-acid-p-sulfo-benzoic-acid-diamide in a caustic soda solution of about 8 per cent is added to a viscose solution capable of being spun in such a quantity, that after spinning and coagulating filaments containing about 10 per cent superpolyamide are obtained. The elasticity of these filaments is far greater than that of pure viscose filaments. The filaments, moreover, possess contrary to the others a wool-like grip and excellent "Bauschelastizität."

The filaments may be dyed by boiling one hour with 2 per cent Acid Anthracene Red 3 BL (Schultz dyestuff tables, year 1932, vol. II, page 187) ratio of the weights of filaments and water 1:50, by adding 10 per cent Glauber salt and 4 per cent formic acid. It is then washed with lukewarm water and afterwards dried. The shades obtained are distinctly darker than on viscose silk without addition of the superpolyamide, whereby the degree of fastness is for both kinds at least the same. If the filaments are dyed in the same way with 2 per cent Palatine Fast Blue GGN (Schultz dyestuff tables, year 1932, vol. II, page 108) by adding 6 per cent formic acid or with 2 per cent Sirius Light Blue BRR (Schultz dyestuff tables, year 1934, vol. I, page 131) by adding 20 per cent Glauber salt, also distinctly darker, but more brilliant shades are obtained than on cellulose free from superpolyamides.

#### Example II

50 parts by weight of N.N'-di-propanecarboxylic-acid-diphenylether-4.4'-disulfonic-acid-diamide



and 6 parts by weight of hexamethylenediamine are condensed as described in Example I. The superpolyamide obtained is soluble in an aqueous alkali solution.

An alkaline solution of said condensation product consisting of hexamethylenediamine and N.N'-dipropane-carboxylic-acid-diphenylether-4.4'-disulfonic-acid-diamide is added to a viscose solution as described in Example I in such a quantity, that the finished filaments spun from the solution contain 15 per cent of the superpolyamide. They are spun in the way usually adapted for pure viscose. The filaments are very elastic and show a wool-like grip. If they are boiled one hour with 2 per cent Fast-Mordant-Blue E (Schultz dyestuff tables, year 1934, supplementary volume I, page 90) ratio of the weights of filaments and water 1:50, by adding 10 per cent Glauber salt and 4 per cent formic acid and, if afterwards treated for 45 minutes with 1 per cent potassium chromate, distinctly darker and also faster shades are obtained than on filaments consisting of superpolyamide-free viscose.

In the same way also foils can be obtained and dyed. They also possess darker shades than foils from pure viscose.

Viscose containing 20 per cent of the condensation product obtained from N.N'-dipentanecarboxylic-acid-diphenylether-4.4'-di-sulfonic-acid-diamide is dyed, by boiling one hour and adding 3 per cent soap, with 1.5 per cent Celliton Fast

Blue BF (Cellitonechtblau BF), concentrated powder, ratio of the weights of filaments and water 1:50. The shades are far darker than those from filaments from superpolyamide-free viscose solution, whereby the degree of fastness for both kinds is very much the same.

#### Example III

An alkaline solution of a superpolyamide consisting of 1 mol N.N'-dipropanecarboxylic-acid-p-sulfo-benzoic-acid-diamide, 1 mol adipic acid and 2 mols hexamethylenediamine is added to a viscose solution capable of being spun in such a quantity, that the finished filaments contain about 20 per cent superpolyamide. The filaments are dyed by boiling one hour with 2 per cent Sirius Fast Blue BRR (Siriuschtblau BRR) (Schultz dyestuff tables, year 1934, supplementary volume I, page 131) ratio of the weights of filaments and water 1:50, by adding 20 per cent Glauber salt. Far darker shades than on filaments consisting of superpolyamide-free viscose are thus obtained.

What we claim is:

1. A process for the manufacture of fibers and foils from a mixture of an alkali-soluble linear superpolyamide containing sulfamide groups and a cellulosic solution selected from the group consisting of viscose and ammoniacal copper oxide cellulose, which comprises adding to the cellulosic solution an alkaline solution of the superpolyamide, the amount of superpolyamide added to the cellulosic solution being at least 5%, based on the cellulose in the solution, forming fibers and foils from the resulting solution and coagulating the fibers and foils in a coagulating bath.

2. A process as in claim 1 in which the cellulosic solution is a viscose solution.

3. A process as in claim 1 in which the cel-

lulosic solution is an ammoniacal copper oxide cellulose solution.

4. A process as in claim 1 in which the cellulosic solution is a viscose solution and the superpolyamide is the condensation product obtained from hexamethylene diamine and N.N'-dipropane-carboxylic-acid-p-sulfo-benzoic-acid-diamide.

5. A process as in claim 1 in which the cellulosic solution is a viscose solution and the superpolyamide is the condensation product obtained from hexamethylene diamine and N.N'-dipropane-carboxylic-acid-diphenyl ether-4.4'-di-sulfonic-acid-diamide.

6. A process as in claim 1 in which the cellulosic solution is a viscose solution and the superpolyamide is the condensation product obtained from one mol of N.N'-dipropane-carboxylic-acid-p-sulfo-benzoic-acid-diamide, one mol of adipic acid and two mols of hexamethylene diamine.

7. A new filament as in claim 1 in which the superpolyamide is the condensation product obtained from hexamethylene diamine and N.N'-dipropane-carboxylic-acid-p-sulfo-benzoic-acid-diamide.

8. A spinning solution comprising as essential ingredients at least 5%, based on the weight of the cellulose, of an alkali-soluble linear superpolyamide containing sulfamide groups, dissolved in a cellulosic solution selected from the group consisting of viscose and ammoniacal copper oxide cellulose.

9. A spinning solution comprising as essential ingredients at least 5% based on the weight of the cellulose in the viscose, of the condensation product obtained from hexamethylene diamine and N,N'-dipropane-carboxylic acid-diphenyl-ether-4,4'-disulfonic acid-diamide, dissolved in a viscose solution.

10. A spinning solution as in claim 8 in which the cellulosic solution is viscose and the superpolyamide is the condensation product obtained from hexamethylene diamine and N,N'-dipropane - carboxylic - acid-p-sulfobenzoic-acid-di-  
amide.

11. A new filament comprising regenerated viscose cellulose containing at least five percent, based on the cellulose, and dissolved in the viscose solution from which the filament is formed, of an alkali-soluble linear superpolyamide containing sulfamide groups, said filament being resistant to wrinkling, wool-like in character and readily dyed by acid and acetate silk dyes.

12. Filaments and foils comprising essentially a mixture of regenerated cellulose derived from a cellulosic solution selected from the group consisting of viscose and ammoniacal copper oxide cellulose, and at least five percent, based on the weight of the cellulose, of an alkali-soluble linear

superpolyamide containing sulfamide groups, the superpolyamide being dissolved in the cellulosic solution, said filaments and foils being resistant to wrinkling, readily dyed by acid and acetate silk dyes and having been obtained by the process of claim 1.

JOACHIM AMENDE.  
WILLIBALD ENDER.

#### REFERENCES CITED

The following references are of record in the file of this patent:

#### UNITED STATES PATENTS

| Number    | Name          | Date           |
|-----------|---------------|----------------|
| 1,864,426 | Gardner       | Jan. 21, 1932  |
| 2,136,928 | Schlack       | Nov. 15, 1938  |
| 2,071,251 | Carothers     | Feb. 16, 1937  |
| 2,130,948 | Carothers     | Sept. 20, 1938 |
| 950,435   | Chavassieu    | Feb. 22, 1910  |
| 2,155,067 | Ubbelohde     | Apr. 18, 1939  |
| 2,224,693 | Picard et al. | Dec. 10, 1940  |
| 2,149,273 | Carothers     | Mar. 7, 1939   |
| 2,191,556 | Carothers     | Feb. 27, 1940  |
| 2,265,559 | Watkins       | Dec. 9, 1941   |
| 2,223,916 | Martin        | Dec. 3, 1940   |